

# UNITED STATES PATENT OFFICE.

PAUL JULIUS, VIKTOR VILLIGER, AND PAUL NAWIASKY, OF LUDWIGSHAFEN-ON-THE-RHINE, GERMANY, ASSIGNORS TO BADISCHE ANILIN & SODA FABRIK, OF LUDWIGSHAFEN-ON-THE-RHINE, GERMANY, A CORPORATION.

## TETRACHLOR-INDIGO AND PROCESS OF MAKING SAME.

955,410.

Specification of Letters Patent. Patented Apr. 19, 1910.

No Drawing.

Application filed November 17, 1909. Serial No. 528,562.

To all whom it may concern:

Be it known that we, PAUL JULIUS, Ph. D., VIKTOR VILLIGER, Ph. D., and PAUL NAWIASKY, Ph. D., chemists, the first and third subjects of the Emperor of Austria-Hungary and the second a citizen of the Swiss Republic, residing, respectively, at Ludwigshafen-on-the-Rhine, Germany, have invented new and useful Improvements in Tetrachlor-Indigo and Processes of Making Same, of which the following is a specification.

Our invention relates to the production of 4.4'.5.5'-tetrachlor-indigo. We have invented a process for its production by the saponification and oxidation of an ester of 4.5-chlor-indoxyl carboxylic acid. Thus, upon operating in this way upon the methyl ester of 4.5-dichlor-indoxyl carboxylic acid, we obtain the new product 4.4'.5.5'-tetrachlor-indigo of a constitution corresponding to the formula



It consists, when dry, of a greenish blue powder which yields a blue solution in cold concentrated sulfuric acid and a blue solution in hot dimethyl anilin. It differs from all known tetrachlor-indigos in that it dyes cotton from a vat exceptionally greenish shades of blue which are fast against washing, light, and chlorin. Moreover, the said shades retain their greenish tint when viewed by artificial light, whereas the other tetrahalogen indigos hitherto described assume a reddish or violet-black tint under similar conditions. Upon being oxidized in aqueous suspension with nitric acid, our 4.4'.5.5'-tetrachlor-indigo yields 4.5-dichlor-isatin which can be recrystallized from glacial acetic acid and thus obtained in the form of red needles which melt at about 247° C.

The following example will serve to illustrate further the nature of this invention and how it can be carried into practical effect, but our invention is not confined to this example. The parts are by weight. In this example we first, for convenience, describe the production of the methyl ester of 4.5-dichlor-indoxyl carboxylic acid.

Introduce, while stirring, two hundred and ninety-two parts of the methyl ester of 3.4-dichlorphenyl-glycin -2-carboxylic acid into a solution of twenty-three parts of sodium in one thousand parts of methyl alcohol, and maintain the whole at seventy degrees centigrade for thirty minutes. Distil off the methyl alcohol, digest the residue with one thousand parts of water and two hundred parts of thirty per cent. acetic acid, and filter off and wash and dry the 4.5-dichlor-indoxyl carboxylic acid ester, which is insoluble in water and is difficultly soluble in most of the common organic solvents. It can be converted into the corresponding indigo coloring matter by boiling two hundred and sixty parts of it with six thousand parts of water and five hundred and eleven parts of caustic potash, for thirty minutes, while passing a current of coal gas through the solution. Then add twelve thousand parts of boiling water to the mixture and pass air through it, at a temperature of about one hundred degrees centigrade, until the oxidation is complete. If desired, the saponification can be carried out in the absence of coal gas.

Now what we claim is:—

1. The process of producing 4.4'.5.5'-tetrachlor-indigo by saponifying and oxidizing an ester of 4.5-dichlor indoxyl carboxylic acid substantially as described.

2. As a new article of manufacture 4.4'.5.5'-tetrachlor-indigo which consists when dry of a greenish blue powder, yields a blue solution in cold concentrated sulfuric acid, and a blue solution in hot dimethyl anilin; it dyes cotton particularly greenish shades of blue, and on oxidation in aqueous suspension by means of nitric acid gives rise to 4.5-dichlor-isatin, which 4.5-dichlor-isatin can be recrystallized from glacial acetic acid and thus be obtained in the form of red needles which melt at about 247° C.

In testimony whereof we have hereunto set our hands in the presence of two subscribing witnesses.

PAUL JULIUS.  
VIKTOR VILLIGER.  
PAUL NAWIASKY.

Witnesses:

J. ALEC. LLOYD,  
W. W. SCHMIDT.